

Jan. 5, 1932.

L. JOHNSON

1,839,789

ROLLING SHEET

Filed Nov. 10, 1927



INVENTOR

Lane Johnson  
his atty,  
Byrnes, Stetson & Hamley

## UNITED STATES PATENT OFFICE

LANE JOHNSON, OF INGRAM, PENNSYLVANIA, ASSIGNOR TO UNITED ENGINEERING & FOUNDRY COMPANY, OF PITTSBURGH, PENNSYLVANIA, A CORPORATION OF PENNSYLVANIA

## ROLLING SHEETS

Application filed November 10, 1927. Serial No. 232,286.

This invention relates to the rolling of sheets or tin plate, and provides a method and apparatus whereby the labor cost for a given production is materially lessened over 5 that required for rolling sheets from sheet bars, and whereby other operating costs are also materially reduced.

In carrying out my preferred method, I 10 preferably first roll an ingot into slabs. This operation can be readily carried out on a regular blooming mill or slabbing mill. The slabs are preferably of uniform cross section, regardless of the size and gage of the sheets to be rolled. These slabs may be read- 15 ily stored or may be passed directly to the next stage in the operation.

In the second stage, the slabs are passed 20 through a hot strip mill and are reduced to strips which are preferably of uniform width, but whose thickness may vary in ac- 25 cordance with the gage or dimensions of the sheets desired.

The strips are sheared into lengths which are generally equivalent to the width of the 25 sheets desired, with, of course, due allowance for scrap. The sheared pieces are passed crosswise through a cold mill or mills so as to produce the break-down sheets. The break-down sheets may then be doubled or 30 paired and passed through a heating furnace, and subjected to the usual hot rolling operations for the manufacture of sheets or tin plate. This last operation, however, is materially simplified because the break- 35 down sheet is, say, only twice as thick as the finished product.

Instead of a hot rolling operation to finish the break-down sheet, cold rolls may be employed to reduce it to final thickness. In 40 either case, the labor cost for the sequence of steps above recited is materially lower than the cost of rolling by the old methods. The handling may be practically all mechanical and the quality of the labor is changed. The 45 percentage of skilled labor required is also materially reduced.

The method is also of great advantage in 50 that it is highly flexible. Sheets of various length, width and gage may be rolled with a minimum of changes in roll settings. The

material at various stages of operation, particularly the slabs, may be stored as desired, and chipping, pickling or annealing operations, or any other operations for imparting special qualities to the finished sheet, may 55 be interposed with but little difficulty.

In the accompanying drawings which illustrate more or less diagrammatically the present preferred embodiment of my invention and certain modifications thereof, 60

Figure 1 is a view showing a plant lay-out for carrying out my process, the final rolling being effected in hot mills,

Figure 2 is a similar view, but showing the sheets passed through the heating fur- 65 naces crosswise instead of lengthwise, and

Figure 3 is a view corresponding to a portion of Figure 1, but showing cold mills for reducing the break-down sheet by cold roll- 70 ing.

Referring first to Figure 1, there is shown a slabbing mill comprising horizontal rolls 2 and edging rolls 3. Slabs S<sub>1</sub> of uniform cross section are produced on this mill. The slabs are cut to length in a shear 4 which is interposed in the roll table 5.

The roll table 5 extends to a hot strip mill, but a transfer mechanism 6 is provided between the shear and the hot strip mill so that the sheared slabs may be carried to storage 80 if desired.

The short slabs may be carried direct from the slab mill to the hot strip mill and rolled with the original heat from the ingot, or they may be reheated, or they may be chipped and reheated. Furnaces 7 are provided for reheating the slabs. These furnaces deliver the heated slabs to the roll table 5 so they may be carried to the hot strip mill. The hot strip mill, as herein illustrated, comprises a series 90 of horizontal roll stands 8 and edging rolls 9. The stands are driven by motors M in the usual way.

The metal issues from the hot strip mill as 95 strips 10. These strips are allowed to cool, and are then cut to short lengths by the shear 11. One of the short lengths is indicated at 12 in Figure 1.

These sheared pieces of strip may be heat 100

treated in any desired way, or they may be pickled, sand blasted or shot blasted.

The short strips are delivered from the shear 11 onto a roll table 13 by which the short strips are carried to a cold mill comprising a plurality of stands 14. The piece 12 is passed crosswise through the stands 14 and issues as a breakdown sheet 15. It will be understood that instead of using a series of stands, as shown in Figure 1, a single stand 10 may be employed and the piece passed through several times.

The stands in the hot strip mill and in the cold mill may be of any type, but it is preferred to employ four high stands in the cold mill, and in at least some of the passes of the hot strip mill.

The break-down strip 15 is carried by a roll table 16 to the vicinity of the heating furnaces 17.

After the matched or doubled break-down sheets leave a furnace 17, they are taken to sheet rolls 18 and are subjected to the usual processes for reducing them to sheets or tin plate. A finished sheet is indicated at F in Figure 1. The sheet rolls 18 are driven in the usual way from a motor M<sub>1</sub> and are provided with the customary drag 19.

In order to more clearly illustrate the process, we may take as an example the rolling of a twenty gage sheet, size 36" x 120". We may start with an ingot 26" wide x 10" thick x 4' long. This ingot will be reduced in the slabbing mill to a slab 3" thick x 24" wide and with a length corresponding to the weight of the ingot. This slab is taken to the shear 4 and cut into shorter slabs, say, 5' long. If desired, the entire slab may be rolled into a strip without dividing it into shorter slabs, although for convenience of handling it will generally be preferred to shear the long slab.

The 3" x 24" slab is rolled in the hot strip mill into a strip 23" wide x .210" thick. This strip is cut by the shear 11 into lengths of 37 1/2". This gives a number of pieces 12, 23" wide, 37 1/2" long and .210" thick. The pieces 12 are then passed crosswise through the cold mill and reduced to break-down sheets 15, these sheets being 37 1/2" wide by 64 1/4" long by .075" thick, or about 14 gage.

The 14 gage break-down sheets are then matched in pairs and passed through the heating furnaces 17 and rolled in the mills 18 to sheets 37 1/2" wide by about 128 1/2" long by .0375" thick, or 20 gage. The sheets are then trimmed to the size wanted, that is to say, 36" x 120".

If it were desired to roll a sheet 36" x 120" by, say, 27 gage, it would only be necessary to double the two sheets obtained by rolling according to the example just given, and finish this pack on the sheet mill, thus 65 producing a pack of four sheets of 27 gage.

As another example, assume that it is desired to make sheets 42" x 120" by 24 gage. We will again make slabs of the same cross section, that is to say, 24" x 3", and these slabs may again be cut to 5' lengths. The 5' slabs will be passed through the hot strip mill so as to produce strips 23" wide x .140" thick, or 10 gage. These strips will be cut to 43 1/2" lengths, and the pieces thus produced will be passed crosswise through the cold mill to produce break-down sheets 43 1/2" wide x 64 1/4" long x .050" thick, or 18 gage. The break-down sheets will be matched or doubled and passed through the sheet or tin plate mill to produce sheets 43 1/2" wide x 128 1/2" long x .025" thick, or 24 gage. These sheets, when trimmed to size in the shears, will give the product desired.

It will thus be seen that sheets of varying size are produced from hot rolled strips which are of substantially the same width, the thickness being varied in accordance with the length and gage of the sheets desired. Wide variations in the product may thus be effected without material changes in the roll settings.

It is of particular advantage to always produce hot strips of uniform width. If the rolls in a hot strip mill are used for narrow strips, they can never be used for wider strips unless the rolls are redressed. On the other hand, considerable variation in the width of the pieces fed to the cold mill may be had without materially affecting their finish.

Figure 2 shows a modified mill lay-out which is similar in all respects to the lay-out of Figure 1, except that the break-down sheets are passed crosswise through the furnaces 17a. A shear 20 for the finished sheets is indicated diagrammatically in this figure.

Figure 3 shows a part of a mill lay-out which differs from that of Figure 1 in that the break-down sheet is reduced to final thickness by the cold rolls. In Figure 3 the pieces 12a which come from the shears 11a are passed through a cold mill comprising stands 14a so as to produce the break-down sheet 15a. The break-down sheet 12a is passed through a series of stands 21 in which it is cold rolled to produce the finished sheet F. These breakdown sheets may be matched or doubled before the second cold rolling, if desired.

The advantages of my invention arise from the fact that the hot strip produced is always of uniform width, thereby materially reducing the necessity for redressing rolls. The variations in width of pieces which are cold rolled is relatively immaterial from this point of view since the finish of the rolls is not so much affected as in the case of the hot mill. Other advantages arise from the simplicity of calculation of the sizes to be rolled at the various stages, and

because of the fact that a wide variety of sizes may be produced with a minimum of change in the setting of the rolls. If we consider the material at various stages of operation from the standpoint of storage, the number of different sizes required is relatively small, thereby simplifying intermediate operations and likewise simplifying the problems of storage and of handling for intermediate operations.

In the appended claims the term "sheets" is used as a term of general definition and not of limitation, and is intended to include sheets employed for the manufacture of tin plate, or other products.

While I have illustrated and described the preferred form of my invention, it will be understood that it may be otherwise embodied or practiced within the scope of the following claims:

I claim:

1. In the method of rolling sheets, the steps consisting in hot rolling a strip, then passing the strip through cold rolls to produce a break-down sheet, and then subjecting the piece to further rolling to reduce it to final thickness.

2. In the method of rolling sheets, the steps consisting in hot rolling a strip, then passing the strip through cold rolls to produce a break-down sheet, and then subjecting the piece to further hot rolling to reduce it to final thickness.

3. In the method of rolling sheets, the steps consisting in hot rolling a strip, then passing the strip crosswise through cold rolls to produce a break-down sheet and then subjecting the break-down sheet to further rolling to reduce it to final thickness.

4. In the method of rolling sheets, the steps consisting in hot rolling a strip, cutting it into pieces whose length is generally the width of the finished sheet, and passing the pieces crosswise between cold rolls.

5. In the method of rolling sheets, the steps consisting in hot rolling a strip, cutting it into pieces whose length is generally the width of the finished sheet, passing the pieces crosswise between cold rolls, and then subjecting the pieces to further rolling to reduce them to final thickness.

6. In the method of rolling sheets, the steps consisting in hot rolling a strip, cutting it into pieces whose length is generally the width of the finished sheet, passing the pieces crosswise between cold rolls, and then subjecting the pieces to further hot rolling to reduce them to final thickness.

7. In the method of rolling sheets, the steps consisting in hot rolling a strip, then passing the strip crosswise through cold rolls, and then matching or doubling the material and subjecting it to further rolling to reduce it to final thickness.

8. In the method of rolling sheets of vary-

ing sizes or gages, the steps consisting in hot rolling strips of substantially uniform width, varying the thickness in accordance with the length and gage of the sheets desired, cutting sections from the strips, the sections being of a length which is generally the width of the finished sheets, and passing the pieces crosswise between cold rolls.

9. In the method of rolling sheets of varying sizes or gages, the steps consisting in hot rolling strips of substantially uniform width, varying the thickness in accordance with the length and gage of the sheets desired, cutting sections from the strips, the sections being of a length which is generally the width of the finished sheets, passing the pieces crosswise between cold rolls, and then subjecting the pieces to further rolling to reduce them to final thickness.

10. In the method of rolling sheets of varying sizes or gages, the steps consisting in hot rolling strips of substantially uniform width, varying the thickness in accordance with the length and gage of the sheets desired, cutting sections from the strips, the sections being of a length which is generally the width of the finished sheets, passing the pieces crosswise between cold rolls, and then subjecting the pieces to further hot rolling to reduce them to final thickness.

11. In the method of rolling sheets of varying sizes or gauges, the steps consisting in hot rolling strips of substantially uniform width whereby marking of the product by the rolls is obviated, varying the thickness in accordance with the length and gauge of the sheets desired, cutting sections from the strips of a length equal to the width of the finished sheets with trimming allowance, and passing the pieces crosswise between cold rolls so as to eliminate marking of the product.

In testimony whereof I have hereunto set my hand.

LANE JOHNSON. 110

115

120

125

130